

Patented Apr. 8, 1924.

1,489,254

## UNITED STATES PATENT OFFICE.

LESTER KIRSCHBRAUN, OF CHICAGO, ILLINOIS.

## COATED WATERPROOF SHEETING.

No Drawing. Original application filed February 1, 1919, Serial No. 274,495. Now Patent No. 1,464,717.  
 Divided and this application filed April 21, 1921. Serial No. 463,364.

To all whom it may concern:

Be it known that I, LESTER KIRSCHBRAUN, a citizen of the United States, residing in the city of Chicago, county of Cook, and 5 State of Illinois, have invented certain new and useful Improvements in Coated Waterproof Sheetings, of which the following is a specification.

This application is a division of an original 10 application filed by me in the United States Patent Office under date of February 1, 1919, Serial No. 274,495.

This invention relates to improvements in coated waterproof coverings, such, for example, as roofing, and has among its salient objects, to provide a waterproof felted sheet, to which is applied fibre-containing adhesive coating; to provide a product in which the body or felted portion is preferably waterproofed simultaneously with the formation of the sheet, although in certain cases the body portion may consist of ordinary saturated felt to which is applied the fibre-containing coating; to provide a 20 product which permits of the use of relatively low melting point asphalt as a coating; to provide a product in which the coating has a maximum stability and in which the asphalt or bitumen is reinforced 25 against flowing by the fibrous constituents; to provide a product in which very cheap fibre of many different kinds can be used, and in general, to provide an improved product and process of the character referred 30 to.

Describing now the preferable way of forming the product of the present invention, I make an aqueous mixture of water and an emulsifying agent, such, for example, as a clay containing a sufficient percentage of colloidal particles. To this mixture, and while it is in a heated condition, is added an adhesive binder while in liquid form, such as melted asphalt or analogous 40 bitumens or pitches. The binder is thoroughly amalgamated with the emulsifying agent and water so as to form an emulsified matrix in which the binder is in the internal phase and the emulsifying agent and water in the 45 external phase. This matrix is then intimately mixed with the fibre in a water vehicle. The matrix above referred to may consist, by weight, of fifty parts binder, forty parts water and ten parts clay. This

mixture, with the fibre added, may be then 55 passed over an ordinary paper or felt machine. As the sheet is formed, the water dries out and the emulsion is broken and the bitumen becomes adhesive and intimately unites with the fibre. The proportion of 60 ingredients in the finished sheet may be as follows: fifty-five per cent of asphalt, eleven per cent of clay and thirty-four per cent of fibre.

After this sheet is formed, as stated, the 65 coating is applied, preferably after the sheet passes over the last drying rolls of the paper machine. The coating mixture, after being formed in the manner hereinafter described, may be applied in the same way 70 as asphalt coating is applied to ordinary saturated felt. The coating in the present invention, as heretofore stated, consists of bitumen and fibre. Preferably, the coating consists of a mixture of an emulsified matrix 75 and fibre formed in the manner heretofore described, except that a much less percentage of fibre is used. For example, the mixture may consist of ten per cent of fibre, the remainder being asphalt and clay. The emulsion is formed for the reason that the coating can thus be applied cold, but it is not desired to felt the coating; rather, the fibre may be said to more or less float through the asphalt, producing thereby a fibred asphalt 80 coating. For example, a coating of this character may, in some cases, use asphalt for as low as 140 melting point, whereas, ordinarily, from 200 to 260 melting point asphalt is used. Various fibres may be used 85 in this coating, such as cheap fibres ordinarily not suitable for making good paper. After the coating is applied, the sheet is run over drying rolls to remove the water. The bitumen then acts in the manner heretofore 90 described. As the water is driven out, the heated bitumen becomes plastic and a granular facing can then be applied to the adhesive coating.

I claim as my invention:

1. A waterproof covering consisting of a felted waterproof fibrous sheet saturated with a bituminous binder and a coating applied to one surface thereof containing bitumen, fibre and an emulsifying agent. 100

2. A waterproof covering consisting of a felted sheet, a coating applied thereto, said coating containing bitumen, and a minor 105

percentage of fibre and an emulsifying agent, and a granular facing adhesively uniting and covering said coating.

3. A waterproof covering consisting of a felted sheet, saturated with a bituminous waterproof binder a coating applied thereto, said coating containing bitumen, and a minor percentage of fibre and an emulsifying agent.
- 10 4. A waterproof covering consisting of a felted sheet saturated with a waterproof binder connected with a substance contain-

ing a major percentage of bitumen and a minor percentage of fibre and an emulsifying agent.

- 15 5. A waterproof covering consisting of a felted sheet saturated with a waterproof binder, coated with a substance containing a major percentage of bitumen and a minor percentage fibre, and an emulsifying agent, <sup>20</sup> and a granular surfacing bonded to the coating.

LESTER KIRSCHBRAUN.